

3,058,818

GASOLINES CONTAINING POLYMERIC  
ADDITIVE AGENTS

Adlai E. Michaels, Cranford, Elbert D. Nostrand, Westfield, and Thomas S. Tutwiler, Watchung, N.J., assignors to Esso Research and Engineering Company, a corporation of Delaware  
No Drawing. Filed Apr. 22, 1959, Ser. No. 807,987  
10 Claims. (Cl. 44—62)

The present invention relates to improvements in the properties of petroleum distillate fuels. It more particularly relates to gasolines which have been improved by the incorporation therein of certain polymeric additive agents which effect a significant reduction in the amount of deposits, sludge and varnish formed in gasoline engines operated upon such fuels.

A primary factor in formation of deposits, sludge and varnish in gasoline engines is incomplete combustion of the fuels introduced into the combustion chambers of such engines. Studies carried out with radioactive tracer materials have shown that certain polynuclear aromatics and other relatively high boiling compounds normally found in gasolines are only partially burned under normal operating conditions. The small but significant quantities of hydrocarbons which remain unburned apparently undergo complex cracking, polymerization, and oxidation reactions in the combustion chamber and form carbonaceous deposits which adhere to the upper part of the cylinder head, the valves, the piston tops and other surfaces with which the hot gases come in contact. Some of these complex reaction products are also apparently blown past the piston rings into the crankcase of the engine where they are dissolved in the lubricating oil. When the oil subsequently comes into contact with hot metal surfaces, the dissolved materials apparently further react to form insoluble products which appear as sludge.

The effects of deposits, sludge and varnish thus formed in gasoline engines are serious ones. Residues accumulated in the combustion chambers are in part responsible for surface ignition, spark plug fouling, rumble, octane requirement increase and other combustion difficulties well known to those skilled in the art. Material accumulated elsewhere in the engine often causes malfunctioning of the engine lubricating system, accelerates the rate at which wear of engine parts occurs, increases engine oil consumption, and results in improper valve and piston ring operation. All of these difficulties produce serious losses in engine power. Engine maintenance expense and engine life are also seriously affected.

The present invention provides a class of new and improved gasolines which are much less susceptible to the formation of engine deposits, sludge and varnish than gasolines employed heretofore. In accordance with the invention, it has now been found that the use of certain selected copolymers of vinyl pyrrolidones and esters of acrylic acids in gasolines greatly improves engine cleanliness, permits economies in engine operation generally unattainable heretofore, and obviates the necessity for certain costly refining process steps which were often necessary in the past in order to produce gasolines with the required cleanliness properties.

The copolymers which are employed as gasoline additives in order to reduce the formation of engine deposits, sludge and varnish in accordance with the invention are copolymers of N-vinyl pyrrolidones and alkyl esters of acrylic and methacrylic acids. Although the mechanism by which these copolymers act to reduce the formation of deposits, sludge and varnish in gasoline engines is not fully understood, it has been found that these particular copolymers possess properties not found in other copoly-

mers of similar structure which have in the past been employed as additives in lubricating oils and similar compositions.

The N-vinyl pyrrolidones which constitute one monomer of the copolymers employed as gasoline additives in accordance with the invention are compounds having the following general formula:

10



15 where the R's represent hydrogen atoms or aliphatic hydrocarbon radicals containing from 1 to 5 carbon atoms each.

Specific examples of such N-vinyl pyrrolidones include N-vinyl pyrrolidone itself, 3-methyl-1-vinyl-pyrrolidone, 4-methyl-1-vinyl-pyrrolidone, 5-methyl-1-vinyl-pyrrolidone, 3-ethyl-1-vinyl-pyrrolidone, 4-ethyl-1-vinyl-pyrrolidone, 3, 3-dimethyl-1-vinyl-pyrrolidone, 3,4-dimethyl-1-vinyl-pyrrolidone, 3,5-dimethyl-1-vinyl-pyrrolidone, 5,5-dimethyl-1-vinyl-pyrrolidone, 3,4-dipropyl-1-vinyl-pyrrolidone, 3,4,5-triisopropyl-1-vinyl-pyrrolidone, 3,4-dimethyl-5-propyl-1-vinyl-pyrrolidone, 4-butyl-1-vinyl-pyrrolidone, 3-amyl-3,5-dimethyl-1-vinyl-pyrrolidone, 3,4,5 - triethyl - 3 - butyl-1-vinyl pyrrolidone, 5,5-diamyl-1-vinyl-pyrrolidone and the like. N-vinyl pyrrolidone itself is particularly effective in preparing the copolymers utilized in accordance with the invention and is therefore preferred.

20 Acrylic esters employed as the second constituent of the copolymers are alkyl esters of acrylic and methacrylic acids having esterifying groups containing from 1 to about 24 carbon atoms. Alkyl esters in which the alkyl groups contain from about 4 to about 18 carbon atoms are particularly useful because of the solubility properties which they impart to the copolymers, and are therefore preferred for purposes of the invention. Examples of such esters which may be employed to prepare the copolymers include butyl methacrylate, n-hexyl methacrylate, dodecyl methacrylate, hexadecyl methacrylate, octadecyl acrylate, eicosyl methacrylate, 2-ethyl-hexyl acrylate, stearyl methacrylate, cetyl acrylate, and the like.

25 Esters of acrylic and methacrylic acids prepared from commercial mixed alcohols may also be used in preparing the copolymers employed in accordance with the invention. Such mixed alcohols include those prepared by the hydrogenation of coconut oil and marketed commercially under the trade name "Lorol." One such mixture of alcohols consists primarily of lauryl alcohols but contains compounds of from about 10 to about 18 carbon atoms per molecule. This particular "Lorol" alcohol normally contains about 4.0% of  $C_{10}$  alcohol, about 55.5% of  $C_{12}$  alcohol, about 22.5% of  $C_{14}$  alcohol, about 14.0% of  $C_{16}$  alcohol, and about 4.0% of  $C_{18}$  alcohol. Tallow alcohol is a similar mixed product consisting primarily of cetyl and stearyl alcohols derived from tallow fat by hydrogenation. Other mixed alcohols available commercially are derived from soybean oil, cottonseed oil, and similar natural products and also have chain lengths within the range recited above which render them suitable for purposes of the invention.

30 A still further class of alcohols which may be employed in preparing the esters used as monomers in accordance with the invention are the oxo alcohols which are derived by the oxonation and hydrogenation of olefin polymers. A variety of alcohols may be produced by this method, depending upon the particular olefins employed. If a  $C_7$  copolymer of propylene and butylene is used, for example,  $C_8$  oxo alcohol is produced. Typically  $C_8$  oxo alcohol consists of 29% of 3,5-dimethyl-

hexanol, 25% of 4,5-dimethylhexanol, 17% of 3,4-dimethylhexanol, 16% of 4-methyl-heptanol and 5-methyl-heptanol, 2.3% of 4-ethyl-hexanol, 1.4% of 5,5-dimethylhexanol, 4.3% of 2-alkyl-alkynols, and 5% of other alcohols. If a propylene tetramer is subjected to oxonation and subsequent hydrogenation, a C<sub>13</sub> oxo alcohol is produced. This higher alcohol consists of a mixture of alcohols similar to the C<sub>8</sub> oxo alcohol mixture. Other alcohols of different chain lengths and different degrees of branching may be produced in similar manner. All of these alcohols are suitable for use in forming the esters employed as one of the monomers of the additives of the invention.

The alkyl acrylates and methacrylates and the N-vinyl pyrrolidones described in the preceding paragraphs are polymerized to produce the copolymers employed in gasolines in accordance with the invention by mixing them in proportions of from about 1 to about 30 weight percent of the N-vinyl pyrrolidone and about 70 to about 99 weight percent of the acrylate or methacrylate ester. Polymerization of the monomers in ratios of from about 5 to about 15 wt. percent of the N-vinyl pyrrolidone and about 85 to about 95 wt. percent of the acrylate or methacrylate ester is preferred. The polymerization reaction may be carried out without diluent or instead may be carried out in a solution of a paraffinic solvent such as heptane or white oil at a temperature in the range of from about 60° F. to about 250° F. Gamma radiation may be used to promote polymerization or instead a peroxide type catalyst such as benzoyl peroxide, a hydro peroxide or an azo catalyst such as  $\alpha$ - $\alpha'$ azo-bis-isobutyronitrile may be employed. It is usually preferred to carry out the polymerization reaction under a blanket of an inert gas such as nitrogen or carbon dioxide in order to exclude oxygen. The polymerization time may vary from about 1 to about 36 hours.

The copolymers produced in the manner described above, may have molecular weights in the range of from about 1000 to about 100,000 or higher Staudinger. It is generally preferred to limit the polymerization reaction so that a product having a molecular weight of from about 2000 to about 20,000 Staudinger is obtained. The copolymer product may be recovered from the polymerization reaction mixture by evaporating off the solvent.

The copolymer thus prepared may be incorporated in the gasolines in concentrations in the range of from about 0.001% to about 2.0% by weight. Concentrations in the range of from about 0.005% to about 0.2% are generally highly effective and are therefore preferred. An effective method for incorporating the copolymers in the gasolines is to employ a solvent such as xylene, a highly refined lubricating oil, a white oil or the like. The copolymers are soluble in gasolines at the concentrations in which they are used in accordance with the invention, however, and hence may be added directly to the fuel without the necessity for using any solvent at all.

The gasolines in which the copolymers are employed in order to reduce the formation of deposits, sludge and varnish are conventional fuels employed in internal combustion engines operating on the Otto cycle. They are supplied in a number of different grades depending upon the type of service for which they are intended. The copolymers may be employed in all of these grades but are particularly useful in motor gasolines. Motor gasolines as referred to in connection with the present invention are defined by ASTM Specification D-439-56T in Types A, B and C. They are composed of a mixture of various types of hydrocarbons including aromatics, olefins, paraffins, isoparaffins, naphthenes and, occasionally, diolefins. They are derived from petroleum crude oil by refining processes such as fractional distillation, catalytic cracking, hydroforming, alkylation, isomerization, polymerization and solvent extraction. Motor gasolines normally have boiling ranges between about 70° F.

and about 450° F. The copolymers may also be employed in aviation gasolines, which have properties similar to those of motor gasolines but normally have somewhat higher octane numbers and narrower boiling ranges. 5 The properties of aviation gasolines are set forth in U.S. Military Specification MIL-F-5572.

The copolymeric additives employed in accordance with the invention may be used in gasolines with other additive agents conventionally used in such fuels. It is 10 conventional practice to employ from about 2 to about 4.6 ccs. of tetraethyl lead, tetramethyl lead, dimethyl-diethyl lead or a similar alkyl lead anti-knock agent in both motor gasolines and in aviation gasolines. Halogenated hydrocarbons and phosphorus compounds are 15 generally employed as scavenger agents in gasolines containing lead anti-knock agents and are used in concentrations ranging from about 0.05 to about 1.0 or more theories of the phosphorus compound and from about 1 to about 3.0 theories of the halogenated hydrocarbons, 20 based on the stoichiometric equivalent of the lead content. Other gasoline additives with which the additives of the invention may be employed include materials designed to stabilize tetraethyl lead and similar anti-knock agents, solvent oils, rust and corrosion inhibitors, 25 anti-icing agents, dyes and dye stabilizers. The additive agents employed in accordance with the invention are non-reactive in gasolines and may be used in conjunction with a wide variety of such conventional gasoline additives.

The nature and objects of the present invention are 30 further illustrated by the results of tests carried out to demonstrate the effectiveness of the copolymeric additives in reducing the formation of sludge, varnish and deposits in gasoline engines. The copolymer employed in the test was a copolymer containing 8 wt. percent of 35 N-vinyl pyrrolidone and 92 wt. percent of a mixture of alkyl methacrylates having an average chain length of 9½ carbon atoms. The mixed alkyl methacrylate contained equal proportions of butyl methacrylates, C<sub>8</sub>-C<sub>10</sub> straight chain methacrylates, "Lorol" methacrylate, and 40 tallow methacrylate. The copolymer had a molecular weight of about 15,000 Staudinger. It was employed as a 38 wt. percent solution in mineral oil.

Two hundredths of 1% of the mineral oil containing 38 wt. percent of the copolymer described above was incorporated 45 into a commercial leaded gasoline to give a copolymer concentration of 0.0076 wt. percent. The gasoline line used had the following properties:

#### Base Gasoline Inspections

|    |                                     |      |
|----|-------------------------------------|------|
| 50 | ASTM distillation, method D-86:     |      |
|    | Initial boiling point, °F-----      | 90   |
|    | 10% boiling point, °F-----          | 131  |
|    | 50% boiling point, °F-----          | 231  |
|    | 90% boiling point, °F-----          | 362  |
| 55 | Final boiling point, °F-----        | 424  |
|    | Reid vapor pressure, p.s.i-----     | 13.5 |
|    | General Motors gum, mg./100 ml----- | 3.2  |
|    | ASTM breakdown time, min-----       | 845  |
| 60 | FIA analysis:                       |      |
|    | Vol. percent saturates-----         | 67.1 |
|    | Vol. percent olefins-----           | 16.3 |
|    | Vol. percent aromatics-----         | 16.6 |
|    | Tetraethyl lead, cc./gal-----       | 2.95 |
| 65 | Research octane No.-----            | 92.5 |
|    | Motor octane No.-----               | 85.5 |

Samples of the base gasoline and samples of the same gasoline containing 0.0076 wt. percent of the copolymer described above were separately employed in a sustained engine test designed to evaluate gasoline performance under varied operating conditions. A 1950 6-cylinder Chevrolet engine attached to a dynamometer on a test stand was operated to the following repeated cycles for 70 a period of about 110 hours.

## Test Conditions

| Cycle | R.p.m. | Jacket Water Outlet Temp., °F. | Oil Sump Temp., °F. | Intake Air, °F. | Brake H. P. | Air/Fuel Ratio | Cycle Duration, Hrs. |
|-------|--------|--------------------------------|---------------------|-----------------|-------------|----------------|----------------------|
| 1     | 500    | 115                            | 115                 | 70              | 0           | 9.5/1          | 1½                   |
| 2     | 2,000  | 160                            | 175                 | 70              | 40          | 11.5/1         | 2                    |
| 3     | 2,000  | 160                            | 215                 | 70              | 40          | 11.5/1         | 2                    |

At the conclusion of the 110 hour period, the engine was inspected and various parts were rated for sludge, deposits and varnish on a demerit scale ranging from 0 to 100, 0 indicating the presence of no deposits at all and 100 signifying that the particular part rated had the maximum amount of deposits it was capable of holding. The results of these ratings are set forth in the following table.

|                               | Demerit Ratings                |                                                            |
|-------------------------------|--------------------------------|------------------------------------------------------------|
|                               | Base Gasoline (A.v. of 2 Runs) | Base Gasoline + 0.076 Wt. Percent Copolymer A <sup>1</sup> |
|                               |                                |                                                            |
| Piston Skirt Varnish, Overall | 79.0                           | 40.8                                                       |
| Thrust Side                   | 79.5                           | 45.0                                                       |
| Anti-Thrust Side              | 78.3                           | 36.7                                                       |
| Ring Zone, Overall            | 14.4                           | 12.8                                                       |
| Sludge, Overall               | 6.9                            | 5.0                                                        |
| Cylinder Head Top             | 5.0                            | 5.0                                                        |
| Rocker Arm Assembly           | 3.7                            | 5.0                                                        |
| Rocker Arm Cover              | 7.5                            | 2.5                                                        |
| Crankshaft                    | 6.2                            | 7.5                                                        |
| Timing Gear Cover             | 12.5                           | 5.0                                                        |
| Push Rod Chamber              | 5.0                            | 7.5                                                        |
| Push Rod Chamber Cover        | 11.2                           | 7.5                                                        |
| Crankcase                     | 0                              | 0                                                          |

<sup>1</sup> Copolymer A was a copolymer of 8 wt. percent N-vinyl pyrrolidone and 92 wt. percent of a mixture of alkyl methacrylates having alkyl groups averaging 9½ carbon atoms in length, 38 wt. percent in mineral oil.

The test results shown in the above table clearly demonstrate that the presence of the copolymer greatly improved the engine performance characteristics of the gasoline. Despite the very low concentration of copolymer used, the sludge and varnish produced when the engine was operated on the fuel containing the copolymer were significantly lower than those obtained when the base gasoline was used. It was further observed that the use of the copolymer gave rise to no spark plug fouling difficulties whatsoever, although spark plugs normally become fouled very readily during the idle cycle of the test. Moreover, the carburetor and other parts of the fuel system were exceptionally clean when the copolymer additive was used, indicating that the copolymer was not deposited out in the carburetor or elsewhere. It was also observed that use of the copolymer reduced engine oil consumption and gave increased power due to better valve operation. These improved results obtained with the copolymeric additive are particularly surprising in view of the fact that the polymers are essentially non-volatile and must enter the combustion chamber of the engine by entrainment in the liquid phase rather than by vaporization.

Additional tests were carried out to determine the effect of the copolymers in other gasolines and at higher concentrations. The copolymer of N-vinyl pyrrolidone and mixed alkyl methacrylates previously described was added as a 38% solution in mineral oil to two leaded gasoline, one a commercial gasoline of regular grade and the other a specially blended gasoline of regular grade volatility known to result in the formation of much more deposits, sludge and varnish than are obtained with commercial fuels. The solution containing the copolymer was added to each gasoline in 0.04 wt. percent concentration, giving a copolymer concentration of 0.015 wt. percent in each fuel. Parallel tests were then carried out using the

gasolines thus prepared and the base gasolines containing no copolymer. The test conditions and procedures employed were the same as those described above. The results of these tests are shown in the following table.

|                               | Demerit Ratings <sup>1</sup> |                                                              |                              |                                                              |
|-------------------------------|------------------------------|--------------------------------------------------------------|------------------------------|--------------------------------------------------------------|
|                               | Base Gasoline A <sup>2</sup> | Base Gasoline A + 0.015 Wt. percent Copolymer A <sup>3</sup> | Base Gasoline B <sup>4</sup> | Base Gasoline B + 0.015 Wt. percent Copolymer A <sup>3</sup> |
| 15                            |                              |                                                              |                              |                                                              |
| Piston Skirt Varnish, Overall | 55.6                         | 44.9                                                         | 87.5                         | 34.6                                                         |
| Thrust Side                   | 65.0                         | 51.6                                                         | 91.7                         | 36.7                                                         |
| Anti-Thrust Side              | 48.3                         | 38.3                                                         | 83.3                         | 32.5                                                         |
| Ring Zone, Overall            | 12.1                         | 10.1                                                         | 18.5                         | 12.3                                                         |
| Sludge, Overall               | 4.2                          | 0.3                                                          | 8.9                          | 1.9                                                          |
| Cylinder Head Top             | 2.5                          | 0                                                            | 5.0                          | 0                                                            |
| Rocker Arm Assembly           | 2.5                          | 0                                                            | 5.0                          | 0                                                            |
| Rocker Arm Cover              | 5.0                          | 0                                                            | 7.5                          | 2.5                                                          |
| Crankshaft                    | 2.5                          | 0                                                            | 7.5                          | 0                                                            |
| Timing Gear Cover             | 10.0                         | 0                                                            | 15.0                         | 2.5                                                          |
| Push Rod Chamber              | 2.5                          | 0                                                            | 15.0                         | 0                                                            |
| Push Rod Chamber Cover        | 10.0                         | 0                                                            | 12.5                         | 5.0                                                          |
| Crankcase                     | 2.5                          | 0                                                            | 10.0                         | 5.0                                                          |
| Oil Screen                    | 0                            | 0                                                            | 2.5                          | 0                                                            |
| 20                            |                              |                                                              |                              |                                                              |
| 25                            |                              |                                                              |                              |                                                              |

<sup>1</sup> Rating indicates amount of sludge, deposits and varnish on part rated, 0 signifying that the part was clean and 100 indicating that the part had the maximum amount of sludge, deposits and varnish it was capable of holding.

<sup>2</sup> Base gasoline A was a regular grade leaded gasoline marketed commercially for use in automobiles.

<sup>3</sup> Copolymer A was a copolymer of 8 wt. percent of N-vinyl pyrrolidone and 92 wt. percent of mixed alkyl methacrylates having mixed alkyl groups averaging 9½ carbon atoms in length, 38 wt. percent in mineral oil.

<sup>4</sup> Base gasoline B was a specially blended gasoline having the same volatility as gasoline A but much less clean-burning than gasoline A.

The data in the above table again demonstrate that gasolines containing the copolymers greatly improve engine cleanliness. The improvement was striking in the case of both gasolines, indicating that the effect is not limited to any particular fuel.

It will be understood that the copolymer composition employed in the foregoing tests is merely representative of the copolymers useful as gasoline additives in accordance with the invention and that other copolymers previously described herein are similarly useful. Examples of such other copolymers are those having the compositions and molecular weights set forth below.

| Monomers in Copolymer                                                                          | Staudinger Mol. Wt. |
|------------------------------------------------------------------------------------------------|---------------------|
| 10 Wt. Percent N-Vinyl Pyrrolidone + 90 Wt. Percent Lauryl Methacrylate                        | 2,500               |
| 5 Wt. Percent 3-Methyl-1-Vinyl Pyrrolidone + 95 Wt. Percent Decyl Acrylate                     | 3,500               |
| 15 Wt. Percent 5,5-Dimethyl-1-Vinyl Pyrrolidone + 85 Wt. Percent Tallow Methacrylate           | 20,000              |
| 17 Wt. Percent 3-Ethyl-1-Vinyl Pyrrolidone + 83 Wt. Percent C <sub>12</sub> -Oxo Methacrylate  | 18,000              |
| 21 Wt. Percent 5-Butyl-1-Vinyl Pyrrolidone + 79 Wt. Percent n-Hexyl Acrylate                   | 32,000              |
| 30 Wt. Percent 3,4-Dimethyl-1-Vinyl Pyrrolidone + 70 Wt. Percent C <sub>12</sub> -Oxo Acrylate | 64,000              |
| 8 Wt. Percent N-Vinyl Pyrrolidone + 92 Wt. Percent "Lorol" Methacrylate                        | 4,200               |
| 19 Wt. Percent 3,4,5-Trimethyl-1-Vinyl Pyrrolidone + 81 Wt. Percent Dodecyl Acrylate           | 10,000              |
| 24 Wt. Percent 3-Amyl-1-Vinyl Pyrrolidone + 76 Wt. Percent 2-Ethyl Hexyl Acrylate              | 7,000               |
| 20 Wt. Percent N-Vinyl Pyrrolidone + 80 Wt. Percent Stearyl Methacrylate                       | 10,000              |
| 25 Wt. Percent 3,3-Dimethyl-1-Butyl-1-Vinyl Pyrrolidone + 75 Wt. Percent Soya Methacrylate     | 16,000              |
| 13 Wt. Percent 3,3-Dimethyl-4,4-Diethyl-1-Vinyl Pyrrolidone + 87 Wt. Percent Nonyl Acrylate    | 21,000              |
| 9 Wt. Percent 3,4,5-Triethyl-1-Vinyl Pyrrolidone + 91 Wt. Percent Methyl Methacrylate          | 3,000               |

<sup>1</sup> Trade name for technical lauryl alcohol.

What is claimed is:

1. A gasoline having incorporated therein from about 0.001% to about 2.0% by weight of a copolymer of from about 1% to about 30% by weight of an N-vinyl pyrrolidone selected from the group consisting of N-vinyl pyrrolidone and alkyl substituted N-vinyl pyrrolidone.

done wherein the alkyl groups have from 1 to 5 carbon atoms and from about 70% to about 99% by weight of an ester selected from the group consisting of alkyl acrylates and methacrylates in which the esterifying alkyl groups contain from 1 to about 24 carbon atoms.

2. A gasoline as defined by claim 1 wherein said ester is an alkyl acrylate.

3. A gasoline as defined by claim 1 wherein the esterifying alkyl groups in said ester contain an average of from 4 to 18 carbon atoms.

4. A gasoline as defined by claim 1 wherein said copolymer is a copolymer from about 5 to about 15 wt. percent of an N-vinyl pyrrolidone and from about 85 to 95 wt. percent of an alkyl methacrylate.

5. A gasoline as defined by claim 1 wherein said copolymer is a copolymer of N-vinyl pyrrolidone and a mixed alkyl methacrylate. 15

6. A gasoline to which has been added from about 0.001% to about 2.0% by weight of a gasoline-soluble copolymer of from about 1% to about 30% by weight of N-vinyl pyrrolidone selected from the group consisting of N-vinyl pyrrolidone and alkyl substituted N-vinyl pyrrolidone wherein the alkyl groups have from 1 to 5 carbon atoms and from about 70% to about 99% by weight of an alkyl methacrylate wherein the alkyl groups 20 contain from 1 to about 24 carbon atoms. 25

7. A gasoline as defined by claim 6 wherein said copolymer is present in a concentration of from about 0.005% to about 0.2% by weight.

8. A gasoline as defined by claim 6 wherein the alkyl groups in said alkyl methacrylate contain from about 4 to about 18 carbon atoms.

9. A gasoline as defined by claim 6 wherein said copolymer is a copolymer of from about 5 to about 15% of N-vinyl pyrrolidone and from about 85 to 95 wt. percent of mixed alkyl methacrylates.

10. A gasoline as defined by claim 6 wherein said copolymer has a molecular weight between about 2000 and about 20,000 Staudinger.

#### References Cited in the file of this patent

##### UNITED STATES PATENTS

|           |                     |               |
|-----------|---------------------|---------------|
| 2,800,452 | Bondi et al. -----  | July 23, 1957 |
| 2,866,729 | Zimpel -----        | Dec. 30, 1958 |
| 2,892,690 | Lowe et al. -----   | June 30, 1959 |
| 2,899,391 | Mayhew et al. ----- | Aug. 11, 1959 |

##### FOREIGN PATENTS

|         |                     |               |
|---------|---------------------|---------------|
| 760,554 | Great Britain ----- | Oct. 31, 1956 |
| 808,665 | Great Britain ----- | Feb. 11, 1959 |